

May 23, 1944.

L. P. MILLER

2,349,511

METHOD OF MAKING CAPSULES

Filed Jan. 28, 1941



FIG. 1



FIG. 2



FIG. 3



FIG. 4

INVENTOR.  
LOUIS P. MILLER

BY *Oberlin, Limbach & Day*  
ATTORNEYS

## UNITED STATES PATENT OFFICE

2,349,511

## METHOD OF MAKING CAPSULES

Louis P. Miller, Cleveland Heights, Ohio, assignor to American Home Products Corporation, Jersey City, N. J., a corporation of Delaware

Application January 26, 1941, Serial No. 376,311

2 Claims. (Cl. 18—57)

The present invention relates to an improved method of making capsules for containing food and pharmaceutical materials, and the like. Such capsules are composed of a water-soluble substance, viz., gelatin, which forms the shell or container, per se, and are filled with a pharmaceutical material. My invention is particularly applicable to the fabrication of such capsules which are adapted to contain liquid or semi-liquid filling materials wherein the gelatin shell is integral and continuous in order properly to seal the material contained therein.

Such capsules of the liquid or semi-liquid filled type are presently made by a process involving first, the formation of the liquid or molten gelatin into solid sheets or bands; secondly, the interposition of the liquid or semi-liquid filling material between two of such sheets; and finally, the pressing together of a "sandwich" of gelatin sheets and filling material between capsule-forming dies whereby portions of the gelatin sheets are deformed or molded into opposed die cavities forming the two halves of the capsule, with the filling material enclosed or trapped therein, and simultaneously sealing or bonding the meeting edges of these two halves together. The problem of properly controlling the physical properties of the gelatin and the gelatin sheets so that they will accommodate the dual functions of being properly and uniformly formed in the die cavities and efficiently bonded or sealed, has been a difficult one in the capsule-making industry. A very close control of the temperature of the gelatin as it passes through the various formation stages from liquid to the completed capsule has been a subject of considerable effort and research. (For example, see article by A. L. Lane in "Electrical World," vol. III, p. 584). It has heretofore been regarded necessary to subject the gelatin sheets or bands, after formation and solidification from the liquid or molten gelatin, to a heating action whereby the adhesive properties and the plasticity of the gelatin is increased in order to obtain a satisfactory forming and sealing or bonding of the halves of the capsule. I have discovered that just the opposite procedure produces the desired results in the forming and bonding ability of the gelatin, and to a greater and more efficient degree than has heretofore been achieved. My invention is, therefore, based upon the unusual and unexpected discovery that the sudden cooling of the gelatin after it is transformed from its liquid state to sheet form and prior to forming and bonding into capsules, produces the physical prop-

erties of flexibility and adhesion which have been so highly desired in the gelatin and result in the increased efficiency and economy of the capsule-making process, as a whole.

To the accomplishment of the foregoing and related ends, said invention, then consists of the steps hereinafter fully described and particularly pointed out in the claims.

The annexed drawing and the following description set forth in detail one approved method of carrying out the invention, such disclosed method, however, constituting but one of various ways in which the principle of the invention may be used.

15 In said annexed drawing:

Fig. 1 is a flow sheet illustrating the various steps of the capsule-making process and with the improvement of my invention as applied thereto; Fig. 2 is an enlarged, detailed sectional view 20 illustrating the step of the process wherein the liquid or molten gelatin is formed into a solid sheet or band; Fig. 3 is another enlarged, sectional view illustrating the "sandwich" of gelatin sheets and filler placed in position between the 25 capsule-forming die plates; and Fig. 4 is a similar view to Fig. 3 but showing the die plates in closed position, wherein the resultant capsule has been formed.

Now referring more particularly to Fig. 1, the 30 first stage of the process involves a provision of a quantity of liquid or molten gelatin which is suitably prepared and contained in a tank or reservoir 1. A temperature in the range of 140° to 160° F. is maintained in the tank 1 to insure the molten state of the gelatin. The liquid gelatin from the tank 1 is next poured upon a sheet-forming surface, such as that of the rotating drum 2. As the liquid gelatin is deposited upon the surface of the drum 2 which is maintained at a temperature of 90° F., it is suddenly and rapidly cooled to a point substantially below its solidification temperature or melting point, by means of a body of cold, refrigerated air, introduced through the duct 3 and led around the periphery of the drum 2 by means of the enclosing housing 4. The range of this cooling temperature is from 45° to 65° F. As the melting point of gelatin is in the range of 120° to 130° F. (depending on its quality) it will be seen that 45 this cooling action results in a very rapid freezing and sudden decrease in the temperature of the liquid gelatin, particularly since the latter is in sheet or film form and, therefore, has a very large area exposed to the action of the cooling air.

Referring particularly to Fig. 2, the manner in which the liquid gelatin, as indicated at 5, flows onto the drum 2 under the pouring gate 6 and is then suddenly cooled and solidified to form the solid sheet 7, is illustrated in greater detail. The stippled and the cross-hatched sections represent the approximate points of formation of the liquid and solid states, respectively, of the gelatin. The solid band or sheet of gelatin 7 is then led to the cutting table or conveyor 8 where it is cut into individual sheets by means of the cutting mechanism 9. One of these individual sheets 10 is placed on the upper face of the lower-forming die plate 11, a quantity of liquid or semi-liquid filling material is deposited from the tank 12 on the surface of the sheet 10 and another individual sheet 14 placed on the top thereof. Thus, a "sandwich" resting upon the top of the lower die plate 11 is formed which comprises outer layers 10 and 14 of gelatin sheets and the intermediate layer of filling material, such as cod-liver oil, a pharmaceutical emulsion or the like.

It will be noted that the sheet 7 of gelatin has a "cold air side" marked A, in Fig. 2, and a "drum side," marked B. It has been found that the manner in which these respective sides A and B of the individual sheets 10 and 14 are placed with respect to each other in the formation of the "sandwich" is an important requisite. Thus, as shown in Fig. 3, the "cold air sides" A of the sheets 10 and 14 respectively, are placed outermost or in a position where they will be contacted by the die plates 11 and 16, and the "drum sides" B of the sheets are placed innermost where they will contact each other.

The lower die plate 11 is then placed in a press 15 and the upper die plate 16 pressed down against it. The die plates 11 and 16 contain a multiplicity of registering die cavities 17 and 18 (usually of cylindrical cross-sectional form), respectively, into which portions of the gelatin sheets 10 and 14, being of the proper and desired flexibility, are deformed and forced to form the two halves 19 and 20 of the capsule, and with the body of filling material 13' trapped therein. The projecting lips or flanges 21 and 22, during the final compression or closing stage of the die plates 11 and 16, force the meeting edges of the molded halves 19 and 20 together, thereby effecting a proper seal or bond between these halves to form a complete, continuous and integral capsule shell. The flanges 21 and 22 also simultaneously cut through the body of the gelatin sheets leaving a piece 23 of reticulated form which is commonly termed the "net."

My above described process of making pharma-

ceutical capsules produces capsules which are of uniform size and capacity. The unexpected and remarkable results in the improvement of the capsule-forming properties of the gelatin sheets, produced according to my process is, of course, an important factor in obtaining this uniformity and control of capsule size. If the sheet is too hard and brittle, it will not properly enter the forming die cavities, and by the same token, if it is too soft or plastic, it will enter the die cavities to a greater than the desired extent.

I am unable to ascribe any scientific theory or principle to the novel results achieved by my invention. Suffice it to say that the sudden cooling of the liquid gelatin as it is transformed from liquid to solid form, and to a temperature well below the solidification temperature of the gelatin, probably imparts a "temperature shock" which has a curing effect upon the gelatin sheet which develops a heretofore unknown property of gelatin, because it has previously been supposed that gelatin is of a thermoplastic nature and requires heating in order to render it elastic and adhesive.

The values given herein for the various temperatures will be understood to be by the way of example, and that in actual practice they may be subject to reasonable variations, all within the proper scope and spirit of my invention.

Other modes of applying the principle of my invention may be employed instead of the one explained, change being made as regards the method disclosed herein disclosed, provided the step or steps stated by any of the following claims or the equivalent of such stated step or steps be employed.

I, therefore, particularly point out and distinctly claim as my invention:

1. In the method of making gelatin capsules the steps which comprise, heating gelatin to a temperature range of about 140° F. to about 160° F., to reduce it to molten form, flowing such molten gelatin onto a sheet forming surface maintained at 90° F., simultaneously cooling the exposed side of the sheet to a temperature of from about 45° F. to about 65° F. while subjecting the surface contacting side of the sheet to a temperature of about 90° F.

2. In the method of making gelatin capsules the steps which comprise heating gelatin to a temperature range of about 140° F. to about 160° F., to reduce it to molten form, flowing such molten gelatin onto a sheet forming surface maintained at 90° F., simultaneously cooling the exposed side of the sheet to a temperature below 65° F., while subjecting the surface contacting side of the sheet to a temperature of about 90° F.

LOUIS P. MILLER.